

*Griggs*

Sept. 29, 1959

H. KEUTH ET AL

2,906,649

HEAT-RESISTANT ELECTRIC INSULATION AND METHOD OF MANUFACTURE

Filed April 6, 1956



Fig.1



Fig.2

HEAT-RESISTANT ELECTRIC INSULATION AND  
METHOD OF MANUFACTURE

Heinz Keuth, Altenfurt, near Nurnberg, and Hans-Werner Rotter and Paul Guillery, Nurnberg, Germany, assignors to Siemens-Schuckertwerke Aktiengesellschaft, Berlin-Siemensstadt, Germany, a corporation of Germany

Application April 6, 1956, Serial No. 592,703

Claims priority, application Germany April 7, 1955

21 Claims. (Cl. 117—230)

Our invention relates to the production of electrically insulating and heat-resistant coatings and films of inorganic material and, in one of its more particular aspects, to thin inorganic coatings which adhere firmly to metal-sheet material so as to permit bending and machining the material without impairing the insulating coating. More specifically, the invention also relates to insulation-coated magnetic steel sheets for the core stacks of transformers, reactors, generators, motors or other electromagnetic apparatus, and to dielectric foils or coatings for capacitor electrodes.

It is among the objects of our invention to provide an insulating layer or coating which can be readily applied to cold metal sheets, which will dry rapidly, particularly while passing through an oven or dryer in continuous operation, and which immediately solidifies to great strength and hardness. The insulating layer or coating must also have a high insulating quality and homogeneity at extremely small thickness, preferably below 10 microns, to secure good space utilization when stacking such insulated sheets of magnet steel.

It is another object to make such insulating coatings capable of resisting mechanical stresses, such as bending and punching, without peeling or scaling off. The coatings are further supposed to be scratch-resistant to prevent being damaged by handling and stacking the coated metal sheets.

Another object is to produce such inorganic insulating coatings which do not scale or peel off the metal sheets when annealing the sheets in a reducing atmosphere, as is needed for certain magnetic sheet materials. The coated sheets in a stack do not stick together when annealing the stack; and the above-mentioned mechanical and electrical properties remain preserved after annealing. Furthermore, the coatings are oil- and water-resistant before and after annealing.

These various objects and desiderata, to our knowledge, have never been conjointly obtaining by the known mica or asbestos coatings heretofore available. However, we have found that many or all of the desired qualities are achieved by proceeding, according to our invention, as described presently.

The raw material for producing our coatings is silica mineral substance generally of the mica group, such as mica proper and mica-like substances such as asbestos, bentonite and other silica minerals, all being aluminum-containing silicates and having in common that they contain water of crystallization.

Included in the group of applicable mica-family substances are the synthetic micas such as fluorine mica. Further appertaining to this group are muscovite (potassium mica), phlogopite or biotite (magnesium micas), lepidolite or zinnwaldite (lithium micas), roscoelite (vanadium mica); also ocellacherite, fuchsite, mariposite, paragonite, pholidolite, anomite, lepidomelan, manganese-phyll, ganophyllite, rubellite (rubellan), culsageite, hal-

lerite, philadelphite, polylithionite, taeniolite, margarite, ephesite and others.

The mica-like or near-mica substances applicable for the purposes of the invention are those minerals that possess a crystalline structural relation to pyrophyllite, such as hydrophyllite, and also the incomplete or altered micas having stratified crystals that are valency-unsaturated and, in most cases, occur with a reduced potassium content and an increased content of water. Appertaining to the latter kind of suitable substances are vermiculite and the hydromicas such as hydromuscovite, leverrierite, guembelite, hydrobiotite, glaucite and seladonite; also the illites which generically comprise the mica-like clay minerals, such as serizite, which in contrast to clay proper do not exhibit intra-crystalline swelling.

Applicable synthetic micas, aside from fluorine mica, are the hydrothermal micas including those in the building-up stage as well as the completely formed crystals.

Using any one or more of such combined water-containing minerals of the mica family as a raw material, we proceed as follows.

The mineral substance is first subjected to heating at a temperature above 100° C. and for a period of time sufficient to expel part of the water of crystallization, preferably a major portion of the combined water but not all of it.

Thereafter the substance is mechanically reduced with in a liquid consisting at least partly, but preferably entirely, of water. The comminution is effected, for instance, by a means of a rapidly rotating hammer mill. Then the particles smaller than one micron are segregated from the resulting product and employed to make the coating. A preferred way of doing this is to permit the product to settle until only particles below the size limit remain in suspension within the top zone of the liquid, whereafter the top zone is decanted. An aqueous dispersion of the desired consistency is then formed of the separated particles, that is, the decanted particles, and the dispersion is deposited onto the metal sheet or other body to be coated. This is done by spreading the dispersion like a varnish or paint with a brush, by spraying, by immersing the body into the dispersion, by electrophoresis or in any other suitable manner. Thereafter the coating is dried. The individual mineral particles then adhere firmly to one another and to the surface of the coated body.

Particularly favorable coatings are obtained if the raw mica is first calcined by heating but only to such an extent that it still retains part of its water of crystallization. During calcination, the mica disintegrated into scales. After further mechanical reduction in water, the resulting product is permitted to settle for such a period of time that only particles of an average size of 0.5 micron remain in suspension. If one plots the frequency of occurrence of particles of a given size versus the particle size to obtain a curve, then this curve steeply declines from higher to lower values when the particle size of one micron is exceeded, whereas the slope of the curve is much less toward the smaller particle sizes.

Mainly for the manufacture of annealing-resistant coatings on sheet metal, it is preferable to add to the dispersion of the small mica particles an inorganic colloid, particularly water glass (sodium silicate). Optimum conditions result if about 20% by weight of water glass of commercial dilution, i.e. of the gravity 1.34, is added to the water.

When no water glass or similar colloid is added so that the finished coating consists of mica particles alone, a smooth coating resistant to incandescent temperature is obtained, but this coating is not sufficiently scratch-resistant for some purposes. On the other hand, when a coating is formed of water glass alone or together

with any of the heretofore customary fillers such as heavy spar (barite), zinc oxide or iron oxide, then the coating cracks when subjected to annealing and turns into a fine dust that can be wiped off. The mixture of both kinds of substances, however, results in a very hard coating which, when annealing the coated bodies, causes neither sticking of the sheets nor cracking or scaling of the coating. Particularly favorable results are obtained with a colloidal dispersion containing 20% by weight of mica fines and an addition of 10% by weight of water glass of commercial dilution (gravity 1.34). The amount of water glass may be smaller or larger than 10%. However, when the water-glass content is too small (below 5%), the coatings are soft, whereas when the water-glass content is too large (above 20%), there may occur a local formation of bubbles and a scaling of the insulating coating after annealing, depending upon the condition of the sheet surface and the annealing conditions.

Due to the addition of water glass to the mica suspension, the somewhat swellable mica and the water glass react with each other in such a manner that a thixotropic gel is produced. With the above-mentioned composition of the mixture, this gel is nevertheless still sprayable because the stream of compressed air used for spraying destroys the gel structure. After the sprayed mixture is deposited on the sheet metal to be coated by insulation, the liquid again assumes the original gel character and produces a thin layer which does not run off and dries rapidly. Such coatings have the appearance of a thin, white and smooth varnish coating. They do not require any particular preparation of the sheet surface, can be applied with the facility of a varnish coating, and have excellent adhesion even on smooth sheet surfaces. Because of the slight thickness of the coatings, a good degree of filling or space utilization by magnetic material within a stack of coated sheets is achieved.

Instead of, or in addition to, water glass, the added inorganic colloids may also consist of bentonite, or wetting agents like Nekal, or binding agents. A much smaller amount of added binding agent is sufficient than in the dispersions heretofore used as an insulating varnish. A varnish or insulating paint poor in binding agents has so far become known only for graphite ground to colloidally fine grain size. Such a paint or varnish, however, serves different purposes, namely for producing a conductive coating, for instance on insulators, non-conductive articles that are to be galvanized or electroplated, and the like. As compared with the known mica dispersions which are processed in the manner of paper manufacture to form sheets of mica, the dispersions according to the present invention are distinguished by a much higher degree of comminution of the small particles. We have discovered that by comminuting the raw material to fines of a much smaller degree of size than heretofore known, a dispersion is obtained which can be used and fabricated as readily and in the same manner as varnish and which affords the production of exceedingly thin coatings.

The drawing shows schematically and on enlarged scale a coated magnetic steel sheet in Fig. 1 and an electric capacitor in Fig. 2.

According to Fig. 1, the steel sheet 1 is coated with an extremely thin layer 2 of mica fines made as described above. The capacitor shown in Fig. 2 is composed of electrodes, of which only three are shown at 3, 4, 5, and of intermediate dielectric coatings 6, 7, 8 of mica fines made as described below.

#### Example 1

Muscovite is calcined at 780° C. for approximately one hour. Subsequently the mica, still in hot condition, is placed into distilled water with a pH value below 6.

The same results are obtained when the mica is permitted to cool before immersing it in water.

Within the water, the mica is reduced by means of a hammer mill rotating at approximately 12,000 rotations per minute. Subsequently the comminuted product is permitted to settle in the water. The coarser particles then sink to the bottom. Particles of smaller grain size remain in suspension within the lower portion of the vessel. In the upper portion of the vessel near the level of the water bath, a pulp is formed consisting of a suspension of mica particles smaller than one micron. This pulp is decanted. The remainder of the pulp can again be subjected to a reducing and settling process as described above, and each time the upper pulp zone containing the mica fines below one micron can be decanted. The decanted pulp contains a large amount of water. It is thickened by evaporating a sufficient amount of water to assume the desired consistency, for instance that of a paint or varnish. The thickened suspension is then applied to the surface of metal sheets in the manner of a paint or varnish as described in the foregoing. The varnish-like coating is permitted to dry. Thereafter the coating remains firmly adhering even if the metal sheets are immersed in water.

#### Example 2

A dispersion of mica fines, obtained according to Example 1 by settling and thickening, was supplied with water glass in an amount sufficient to produce a thixotropic liquid. Commercial water glass of 1.34 gravity was used. The composition of the gel-like dispersion was about 20% by weight of mica fines, about 10% water glass and about 70% water. The liquid was applied to sheet metal by means of a spray pistol. After drying of the coating, the sheet metal was annealed at 600 to 800° C. The resulting coating was resistant to scratching, and did not scale off when subjecting the sheet to bending and punching.

#### Example 3

The thickened dispersion produced in accordance with Example 1 and having a pH value of approximately 5 is placed into a vat. A metal sheet to be coated was immersed in the vat and was connected to one pole of a voltage source. An electrode was placed opposite the sheet to be coated. The electrode had a shape and size similar to the sheet and was connected with the other pole. Current was passed through the dispersion between sheet and electrode to electrophoretically precipitate the mica fines upon the sheet. The result was a dense white layer whose thickness is dependent upon the time period of the current supply and the applied voltage as well as upon the electric resistance of the dispersion.

In the manner exemplified by Example 3, coatings of any desired small thickness between 3 to 10 microns, as well as considerably thicker layers, can be produced. Particularly with very thin coatings, the precipitation, after drying, exhibits the properties of a smooth varnish coating which can be heated to glowing temperatures without scaling off.

When the body to be coated, for instance a sheet or tape of metal, is drawn through the electrolyte, such coatings can be produced in a continuous method.

If the precipitated coating is given sufficient thickness and if copper is used as the body or electrode upon which the mica particles are precipitated, then, after drying, the coating can be peeled off as an independent, firmly coherent layer. In this manner, thin heat-resistant insulating foils are produced as are often required for electrical apparatus. For instance, such foils are applicable as a dielectric for capacitors. However, the dielectric layer may also be precipitated directly upon the capacitor electrode in the manner described in the foregoing. Electrode tapes for capacitors, alternating with the above-mentioned foils, can be wound up to form capacitors.

The above-mentioned electrodes directly coated with mica can likewise be given the form of a tape and can be wound up to form capacitors without impairment of the insulating coating.

Another way of producing electric capacitors according to the invention is as follows: At first a capacitor electrode (3 in Fig. 2) is provided with a mica coating 7 as described above. Any necessary terminal means such as conductive strips of foil may then be added. Thereafter another electrode layer 4 is produced on the insulating coating by spraying metal onto the coating. The metal layer is then again coated with insulating material of mica fines 8 according to the invention, and so forth.

Particularly suitable are coatings according to the invention, especially coatings of extreme thinness, for magnetic sheets with preferred magnetic orientation, which in one direction have a considerably higher magnetic permeability than in the direction perpendicular thereto. The good magnetic properties of such sheets are greatly impaired by mechanical fabrication, for instance when the sheets are punched or cut. These properties, however, can be restored by subsequent annealing. The insulating coatings according to the invention, as mentioned, readily withstand the machining or other fabrication of the sheets as well as the annealing. The sheets can be annealed in stacks because, as likewise mentioned, the insulating coatings according to the invention prevent the sheets from sticking together.

We claim:

1. The method of producing upon a metallic surface structure a thin varnish-like, heat-resistant and electrically insulating, inorganic coating having good coherence without an additional binding agent, comprising the steps of partially calcining a mica-group mineral by heating to a temperature and for a length of time sufficient to expel only a part, but a major part, of its water of crystallization, mechanically comminuting said mineral within an aqueous liquid which is weakly acid with a pH of approximately 5 to 6, separating from the comminuted product by decanting the particles smaller than one micron in said weakly acid aqueous liquid, forming an aqueous dispersion containing said liquid and said particles, covering a metal surface structure with a layer of said dispersion, and drying the layer to produce the heat-resistant coating.

2. The method according to claim 1, wherein the liquid of said aqueous dispersion consists of approximately 80% water and about 20% water glass of commercial dilution.

3. The method of producing a thin, varnish-like, heat-resistant, electrically insulating inorganic coating, comprising the steps of heating a crystalline silica mineral of the mica group to expel only part, but a major part, of its water of crystallization, at not higher than about 780° C., mechanically reducing the mineral within aqueous liquid which is weakly acid with a pH of approximately 5 to 6, permitting the resulting product to settle until the particles remaining in dispersion are smaller than one micron, decanting the dispersion, covering a metal surface structure with a layer of the dispersion, and drying the layer to produce the heat-resistant coating.

4. The method of producing a thin, varnish-like, heat-resistant, electrically insulating inorganic coating, comprising the steps of partially calcining by heating a mica-group mineral to expel only part of its water of crystallization, mechanically reducing the mineral within aqueous liquid which is weakly acid with a pH of approximately 5 to 6, permitting the resulting product to settle in the liquid until the particles remaining in dispersion have an average size of 0.5 micron, decanting the dispersion, separating part of the water from the dispersion to obtain a material of varnish-like consistency, covering a metal surface structure with the material to produce thereon the heat-resistant coating upon drying of the ma-

terial, the amount of dispersion applied to the metal surface being limited to that required to form a layer between about three to ten microns thick, the method being carried out at temperatures not higher than about 800° C.

5. The method of producing a heat-resistant coating on a metallic surface structure, comprising the steps of incompletely calcining a swellable mica-group mineral to expel only a portion of its water of crystallization, mechanically reducing the mineral, until at least a portion thereof is under one micron, within an aqueous liquid which is weakly acid with a pH of approximately 5 to 6, separating from the reduction product a dispersion of said weakly acid liquid with particles of the incompletely calcined mineral which are no larger than one micron, adding an inorganic colloid to the aqueous dispersion to form with said dispersion a thixotropic gel material of varnish-like consistency, applying said thixotropic gel material to a surface structure to form a layer thereon, whereby during said applying step said thixotropic material loses the character of a gel and converts to a sol, said material again assuming the character of a gel after it is deposited on said surface structure.

6. The method according to claim 5, wherein said inorganic colloid is water glass.

7. The method of producing a thin, varnish-like, heat-resistant, electrically insulating inorganic coating on metal, comprising the steps of expelling only part of the combined water from muscovite, comminuting the muscovite within aqueous liquid which is weakly acid with a pH of approximately 5 to 6, separating from the reduction product the particles smaller than one micron, forming a weakly acid aqueous dispersion of the separated particles, coating the metal with the dispersion, drying the coating on the metal and subjecting it to annealing temperature.

8. The method of producing a heat-resistant coating on a surface structure, comprising the steps of incompletely calcining a swellable mica-group mineral to expel only a portion of its water of crystallization, mechanically reducing the mineral, until at least a portion thereof is under one micron, within an aqueous liquid which is weakly acid with a pH of approximately 5 to 6, separating from the reduction product a dispersion of said weakly acid liquid with particles of the incompletely calcined mineral which are no larger than one micron, removing part of the water from the dispersion, adding water glass in an amount smaller than the remaining water to form with said dispersion a thixotropic gel material, applying said thixotropic gel material to a surface structure to form a coating layer thereon, whereby during said applying step said thixotropic material loses the character of a gel and converts to a sol, said material again assuming the character of a gel after it is deposited on said surface structure, drying said coating layer, and heating the coated surface structure to a temperature between about 600° and 800° C.

9. The method of producing upon a metallic surface structure a thin varnish-like, heat-resistant and electrically insulating, inorganic coating having good coherence without an additional binding agent, comprising the steps of partially calcining a mica-group mineral by heating to a temperature and for a length of time sufficient to expel only a part, but a major part, of its water of crystallization, mechanically comminuting said mineral within an aqueous liquid which is weakly acid with a pH of approximately 5 to 6, separating from the comminuted product by decanting the particles smaller than one micron in said weakly acid aqueous liquid, forming an aqueous dispersion containing said liquid and said particles, immersing in the dispersion a surface structure to be coated, depositing on said surface structure by electrophoresis a coating from said dispersion, and drying the coating on the surface structure.

10. The method of producing on dynamo steel sheets an electrically insulating thin coating resistant to in-

candescence temperature, comprising the steps of partially calcining by heating mica to liberate only part of its combined water at not higher than about 780° C., mechanically reducing the mica in water which is weakly acid with a pH of approximately 5 to 6, permitting the comminution product to settle until only fines of less than one micron grain size remain in dispersion, decanting the dispersion, evaporating part of the water, adding water glass in an amount less than the remaining water, coating the resulting dispersion product onto the dynamo steel sheets, drying the coatings on the sheets, and subjecting the coated sheets to annealing at a temperature between about 600° and about 800° C., the amount of dispersion applied to the metal surface being limited to that required to form a layer between about three to ten microns thick.

11. The method of dielectrically coating an electrode tape for electric capacitors, which comprises the steps of partially calcining by heating mica to expel only part of its combined water, mechanically reducing the mica in water which is weakly acid with a pH of approximately 5 to 6, permitting the comminution product to settle until only fines of less than one micron grain size remain in dispersion, decanting the dispersion, evaporating part of the water therefrom, passing the electrode tape through the dispersion and applying electric potential between the tape and an electrode to precipitate by electrophoresis a coating onto the tape, and drying the coating.

12. The method of producing inorganic electrically insulating heat-resistant foils, which comprises the steps of partially calcining by heating a mica mineral to expel only part of its combined water, mechanically reducing the mineral within aqueous liquid which is weakly acid with a pH of approximately 5 to 6, separating from the reduction product the particles smaller than one micron, forming an aqueous dispersion of the separated particles, covering a surface structure with a layer of the dispersion, drying the layer, and peeling the layer off the surface structure.

13. The method according to claim 12, wherin the surface structure consists of copper.

14. In combination, a metal body and a heat-resistant varnish-like insulating coating on said body, said coating consisting substantially of dispersed particles of mica all smaller than one micron, said particles retaining part of their original water of crystallization, and said coating having a thickness of about three to about ten microns.

15. In combination, a metal body and a heat-resistant insulating coating on said body, said coating consisting substantially of dispersed particles of mica all smaller than one micron in mixture with water glass, said particles retaining part of their original water of crystallization, said coating being about three to about ten microns thick.

16. A magnetic steel sheet having an insulating coating consisting of a thixotropic dispersion of mica particles of less than one micron particle size in water glass, said layer being about three to about ten microns thick.

5 17. An electric capacitor having a tape electrode coated with a thixotropic layer of a mixture of mica particles and water glass, said particles having all a size below one micron, and said layer being about three to about ten microns thick.

10 18. The method of electrically insulating metal sheets comprising applying thereto an aqueous dispersion which is weakly acid with a pH of approximately 5 to 6 of finely divided particles of a partially calcined mica mineral, the particles having an average size of 0.5 micron and part of their original water of crystallization, the dispersion being thixotropic and containing between 5 and 20 percent by weight of water glass, and thereafter drying and annealing the coated sheet.

15 19. The method of electrically insulating metal sheets comprising applying thereto a coating comprising an aqueous dispersion which is weakly acid with a pH of approximately 5 to 6 of finely divided particles of a calcined mica mineral having an average size of 0.5 micron and part of their original water of crystallization, the particles having a maximum size of not more than one micron, the dispersion being thixotropic and containing between 5 and 20 percent by weight of water glass, and thereafter drying the coated sheets, the amount of dispersion applied being limited to that required to form a layer between about three to ten microns thick.

20 20. The method of electrically insulating metal sheets comprising applying thereto a thin coating comprising an aqueous dispersion which is weakly acid with a pH of approximately 5 to 6 of finely divided particles of a partially calcined mica mineral having an average size of 0.5 micron and part of their original water of crystallization, the particles having a maximum size of not more than one micron, the dispersion containing sufficient water glass 25 to produce a thixotropic liquid, the amount of dispersion applied being limited to that required to form a layer between about three to ten microns thick, and thereafter drying the coated sheet.

25 21. The method of claim 20 in which the mineral is 30 mica.

35 40 21. The method of claim 20 in which the mineral is mica.

#### References Cited in the file of this patent

#### UNITED STATES PATENTS

|    |           |                    |                |
|----|-----------|--------------------|----------------|
| 45 | 686,930   | Heard et al. ----- | Nov. 19, 1901  |
|    | 1,310,939 | Bancroft -----     | July 22, 1919  |
|    | 1,578,813 | Dawes et al. ----- | Mar. 30, 1926  |
|    | 1,867,362 | Lathrop -----      | July 12, 1932  |
|    | 1,963,276 | Miner et al. ----- | June 19, 1934  |
| 50 | 2,076,898 | Labus et al. ----- | Apr. 13, 1937  |
|    | 2,081,935 | Jones -----        | June 1, 1937   |
|    | 2,215,295 | Morrill -----      | Sept. 17, 1940 |
|    | 2,745,141 | Brennan -----      | May 15, 1956   |

#### FOREIGN PATENTS

|    |         |                     |               |
|----|---------|---------------------|---------------|
| 55 | 738,357 | Great Britain ----- | Oct. 12, 1955 |
|----|---------|---------------------|---------------|